

# United States Patent Office

2,930,693

Patented Mar. 29, 1960

1

2,930,693

## PHOTOGRAPHIC MATERIALS CONTAINING N-SUBSTITUTED PHTHALIMIDE COMPOUNDS

Karl Otto Ganguin, and David William Crichton Ramsay, Manchester, England, assignors to Imperial Chemical Industries Limited, London, England, a corporation of Great Britain

No Drawing. Application October 30, 1956  
Serial No. 619,137

Claims priority, application Great Britain  
October 19, 1956

4 Claims. (Cl. 96—66)

This invention relates to photographic materials and more particularly to light-sensitive photographic materials containing developers.

In the usual commercial process for developing exposed photographic materials, the photographic materials are passed through a tank containing the developer in solution. With repeated use of the developer solution, the concentration of the developer falls so that the processing conditions vary and it is eventually necessary to add new developer to the tank. Also when multilayer photographic materials are developed in this way, the developer solution has to diffuse through the upper layers of the photographic materials before it can reach the lower layers so that an even development of the various layers cannot be achieved. For example with a photographic material containing three differently sensitised gelatino silver halide emulsion layers, correct development of the bottom layer can only be obtained by having a high concentration of developer in the developer solution, but under these conditions there is a tendency for the top layer to be over-developed.

Various suggestions have been made to overcome these difficulties. For example, it has been proposed to incorporate in the light-sensitive emulsion layers certain developers, or mixtures of developers with certain stabilisers, and, after exposure, to develop the emulsion layers with aqueous alkali but no such process has yet proved satisfactory in commercial practice.

We have now found that certain substituted phthalimides, as hereinafter defined, can be incorporated in gelatino-silver halide emulsion layers, and that the emulsion layers, after exposure to light can be developed by treatment with an alkaline solution of hydroxylamine or hydrazine which diffuses readily into the emulsion layers of a multilayer material.

According to our invention we provide a light sensitive gelatino-silver halide emulsion layer which contains a substituted phthalimide of the formula



wherein R<sub>1</sub> and R<sub>2</sub> are substituted or unsubstituted alkyl radicals or R<sub>1</sub> and R<sub>2</sub> may be joined together or each or both joined to the benzene ring to form with the nitrogen atom a heterocyclic ring, X is hydrogen, an alkyl, substituted alkyl, alkyloxy, substituted alkyloxy, amino or substituted amino radical, and Y is a solubilising group, and wherein the benzene nuclei may carry substituents.

The solubilising group may be for example a carboxylic or sulphonic acid group or a salt of one of these, for example an alkali metal or ammonium salt.

2

The substituted phthalimides may be made by heating an amine of the formula



wherein R<sub>1</sub>, R<sub>2</sub> and X have the meaning given above and the phenyl nucleus may carry further substituents, with phthalic anhydride or a substituted phthalic anhydride, and, where both the amine and phthalic anhydride are free from water solubilising groups, further treating the product to introduce a water solubilising group.

As examples of the substituted phthalimides which may be used in our invention there may be mentioned the compound made by condensing 4-diethylaminoaniline with trimellitic anhydride (for example by heating the reagents together in boiling glacial acetic acid for 3 hours), the corresponding amino compound (X=NH<sub>2</sub>) formed by nitration and reduction, the compound made by condensing 4-amino-3-ethoxy-N:N-diethylaniline or 4-amino-3-methyl-N:N-diethylaniline with trimellitic anhydride or by condensing 4-diethylaminoaniline or 4-amino-3-ethoxy-N:N-diethylaniline with 4-sulphophthalic anhydride.

In a preferred form of our invention the gelatino-silver halide emulsion layer also contains a colour coupler.

The emulsions used for forming the layers of our invention may be made by simply mixing an aqueous solution or dispersion of the substituted phthalimide with a normal gelatino-silver halide emulsion prepared in the known manner and if desired adding one or more sensitizers, colour couplers and other adjuvants before or after the mixing step. The solution or dispersion of the substituted phthalimide may if desired contain gelatine and/or a surface active agent.

The emulsions may be applied to a film base or paper-base by any known method, for example by dip-coating and subsequent drying.

The emulsion layers of our invention are especially valuable for multilayer colour photographic material and a multilayer colour photographic material wherein at least one of the layers is a gelatino-silver halide emulsion layer containing a substituted phthalimide as hereinbefore defined, forms a further feature of our invention.

Photographic materials containing the light-sensitive emulsion layers of our invention may be exposed to light in the normal way and then developed with an alkaline solution containing hydroxylamine or hydrazine and this process of development forms a further feature of our invention. If desired other adjuvants for example sodium sulphite and potassium bromide may be added to the developer solution. The material may then be fixed and, when the emulsion layer contains a colour coupler, the developed silver may be bleached.

The invention is illustrated but not limited by the following example in which the parts are by weight:

60

### Example

100 parts of a gelatin-silver iodo-bromide emulsion containing 7.25% of gelatin, 3.35% of silver bromide and 0.05% of silver iodide are stirred and there are added 3 parts of a 0.05% solution in methanol of bis-(3-ethyl-5-phenyl benzoxazole-2)-9-ethyltrimethin-cyanine iodide (the iodide of the green sensitising dye-stuff Rr340 described in B.I.O.S. Final Report No. 1355, page 86). The mixture is stirred at 40° C. for 20 minutes and there are then added 24 parts of a 5% aqueous solution of the sodium salt of 4-(omega-cyano-acetyl)-octadecenyl-succinanilide (the colour coupler Kō

302 described in B.I.O.S. Final Report No. 1355, page 75).

The pH of the emulsion is adjusted to 4.7 by the addition of 1.52 parts of a 50% aqueous solution of citric acid, and then 24 parts of an aqueous dispersion containing 1% of gelatine, 0.2 part of sodium diethylsulphosuccinate and 2 parts of 4(4'-carboxy-phthalimido)-3-ethoxy-N:N-diethylaniline are added. The emulsion is coated on a paper base and dried.

The photographic paper so obtained is exposed to the light from an object and then developed in a solution of the following composition:

|                                  | Parts |
|----------------------------------|-------|
| Sodium sulphite, anhydrous       | 1     |
| Hydroxylamine hydrochloride      | 2     |
| Sodium carbonate, anhydrous      | 30    |
| Potassium bromide                | 0.5   |
| Water to make up to 1,000 parts. |       |

The paper is washed and then transferred to a stop bath of the following composition:

|                                  | Parts |
|----------------------------------|-------|
| Sodium thiosulphate              | 200   |
| Sodium sulphite, anhydrous       | 2     |
| Sodium acetate                   | 20    |
| Glacial acetic acid              | 10    |
| Water to make up to 1,000 parts. |       |

The paper is washed and the developed silver is bleached and fixed in a solution of the following composition:

|                                                  | Parts |
|--------------------------------------------------|-------|
| Ferric salt of ethylenediamine-tetra-acetic acid | 20    |
| Sodium carbonate, anhydrous                      | 2     |
| Sodium salt of ethylenediamine-tetra-acetic acid | 10    |
| Sodium sulphite, anhydrous                       | 4     |
| Potassium bromide                                | 10    |
| Sodium thiosulphate                              | 100   |
| Water to make up to 1,000 parts.                 |       |

The paper is finally washed and dried.

What we claim is:

1. A light sensitive gelatino-silver halide emulsion which contains a substituted phthalimide of the formula:



wherein R<sub>1</sub> and R<sub>2</sub> are alkyl radicals, X is selected from the group consisting of alkyl, alkoxy and amino and Y is a

50

solubilising group selected from the class consisting of sulphonic and carboxylic acid groups.

2. A light sensitive gelatino-silver halide emulsion according to claim 1 which contains, in addition to the substituted phthalimide as defined in claim 1, a colour coupler capable of coupling with the oxidation product of a primary aromatic amino developer to form a dye.

3. A photographic material comprising a plurality of layers coated on a support, at least one of said layers being a light sensitive gelatino-silver halide emulsion layer which contains a substituted phthalimide of the formula:



wherein R<sub>1</sub> and R<sub>2</sub> are alkyl radicals, X is selected from the group consisting of alkyl, alkoxy and amino and Y is a solubilising group selected from the class consisting of sulphonic and carboxylic acid groups, and which further contains a colour coupler capable of coupling with the oxidation product of a primary aromatic amino developer to form a dye.

4. A colour photographic process which comprises imagewise exposing to light a light sensitive gelatino-silver halide emulsion which contains a substituted phthalimide of the formula:



wherein R<sub>1</sub> and R<sub>2</sub> are alkyl radicals, X is selected from the group consisting of alkyl, alkoxy and amino and Y is a solubilising group selected from the class consisting of sulphonic and carboxylic acid groups, and subsequently developing with an alkaline solution of a member of the class consisting of hydroxylamine and hydrazine.

#### References Cited in the file of this patent

##### UNITED STATES PATENTS

- 2,137,785 Sanders-Dolgoruki et al. \_\_ Nov. 22, 1938  
 2,478,400 Jelley et al. \_\_ Aug. 9, 1949  
 2,706,157 Sainsbury et al. \_\_ Apr. 12, 1955

##### OTHER REFERENCES

- H. Bennett: "Concise Chemical & Technical Dictionary," page 26, Chemical Publ. Co., Inc., New York, N.Y., publishers (1947).